

Oct. 15, 1940.

H. D. BROWN

2,217,665

PROCESS AND MEANS FOR RECOVERING VANADIUM AND URANIUM FROM ORES

Filed Aug. 22, 1938



INVENTOR.

HARRY D. BROWN.

*H. D. Brown*

ATTORNEY.

Patented Oct. 15, 1940

2,217,665

UNITED STATES PATENT OFFICE

2,217,665

PROCESS AND MEANS FOR RECOVERING  
VANADIUM AND URANIUM FROM ORES

Harry D. Brown, Palisade, Colo.

Application August 22, 1938, Serial No. 226,086

1 Claim. (Cl. 23—18)

This invention relates to a process and to the means for carrying out the process for treating carnotite and other vanadium-uranium ores for the recovery of the vanadium and/or uranium values therefrom.

The principal object of the invention is to provide a continuous process by means of which the values may be extracted at a minimum of cost. Another object of the invention is to provide a highly efficient treating mechanism which will continuously and successively reduce or roast the ore, then immediately oxidize the hot roast in the presence of heat and moisture; thence collect the oxidized ore and deliver it to a continuous cooling apparatus.

Other advantages result from the improved process and the apparatus employed in carrying out the process. These will become more apparent from the following description.

20 In the following detailed description of the invention reference is had to the accompanying drawing which forms a part hereof. Like numerals refer to like parts in all views of the drawing and throughout the description.

25 In the drawing:

Fig. 1 is a longitudinal section through the improved treatment apparatus which is employed in carrying out the improved process.

Fig. 2 is a vertical cross section therethrough taken on the line 2—2, Fig. 1.

30 Fig. 3 is a detail section taken on the line 3—3, Fig. 1.

The apparatus consists of a masonry furnace structure 12 lined with fire brick or other fire-resisting material. A fire box or oxidizing chamber 13, a precipitating chamber 14, and a convection chamber 15 are contained within the furnace structure. The oxidizing chamber is separated from the precipitating chamber 14 by means of a hollow back wall 37 in which there is a relatively low fire arch 16. A stack 17 conveys the combustion gases from the far end of the convection chamber 15.

45 A rotating ore drum 10 extends completely throughout the length of the convection chamber 15 and is supported on the exterior of the furnace upon suitable bearing rollers 11. The drum 10 is provided at one extremity with a feed hopper 18, communicating with the drum 50 through a hollow trunnion 19, and at its other extremity carries an enclosed discharge chute 20. The drum is rotated from any desired source of power through the medium of a suitable drive sprocket 21 and is provided throughout its interior with a conveyor screw 22 and on its exterior

with inclined conveyor paddles 23, which extend in a close proximity to the walls of the chamber 15.

5 A settling passage 24 opens from the bottom of the convection chamber 15 adjacent the precipitating chamber 14. This passage extends downwardly in the back wall 37 and separates to each side of the arch 16 into the side walls of the furnace opening to the latter beneath the arch and above a pair of screw conveyors 25 10 which extend throughout the length of the bottom of the furnace structure.

The conveyors 25 are of the usual hollow shaft type and are water cooled by passing water from a water supply 26 through the hollow conveyor 15 shaft 28. The conveyors are driven from any suitable source of power through drive sprockets 29 and rotate in a direction to convey material to an inclined ore passage 30 leading to a revolving cooling drum 31.

20 A gas or oil burner 32 is positioned at one extremity of the oxidizing chamber 13 so as to blow a flame therein. This burner may be of any suitable type to which fuel is furnished through a fuel pipe 33 and air is furnished through an air pipe 34.

25 Steam jets 35 are also directed into the oxidizing chamber immediately below the chute 20. A steam plate 36 is positioned below the chute 20, and directly under the steam jets 35, to receive 30 the roasted material from the roaster 10.

Operation

35 Before being fed to the roaster, the ore is intermixed with a suitable reagent in predetermined proportions. The particular reagent employed depends upon whether the recovery is to be vanadium alone or both vanadium and uranium. The choice, of course, depends upon the particular ore being worked, as to whether there is sufficient uranium therein to warrant extraction. If both vanadium and uranium are to be extracted, sodium chloride and/or sodium carbonate are used. Should vanadium be the only product to be extracted, the sodium chloride alone is preferred 40 as the reagent.

45 The ore containing the proper percentage of the chosen reagent is fed into the hopper 18 from whence it flows into the decrepitating drum or chloridizing roaster 10 through which it is slowly 50 conveyed by means of the screw 22. The heat in the convection chamber 15 and the speed of travel of the ore are regulated to effect a substantially complete decrepitation or pulverization of the ore before it is delivered to the discharge chute 55

20. The drum is sealed to provide a non-oxidizing atmosphere.

During its travel through the roaster, the ore is decrepitated by the dehydrating action of the 5 heat and the impacts imparted by the cascading rotating action so that preliminary grinding costs are greatly reduced. The ore discharges into the receiving chute 20 at a temperature of approximately 750° F. From the chute, it falls 10 upon the steam table 36 into the steam blasts from the jets 35, which instantly blow the hot ore into the oxidizing flame in highly dispersed condition intermixed with the water particles in the steam. The flame within the oxidizing chamber 15 produces a temperature of approximately 2000° F. which completely oxidizes and calcines 15 the ore and decomposes the steam to furnish additional oxidizing oxygen.

The combustion gases, with the suspended ore 20 particles are deflected downward by the back wall 37 through the restricted opening below the arch 16. This throws a portion of the suspended oxidized ore or dust downwardly onto the conveyors 25. The gases then enter the precipitating chamber 14 where they expand and lose velocity so as to release the remaining suspended dust to the conveyors 25. The gases then rise to and flow through the convection chamber 15 to the stack 17. Any remaining ore dust in the gases will be 30 dropped in the convection chamber and will be conveyed back by means of scrapers 23 to the settings passage 24 from whence it will fall downwardly around the arch 16 to the conveyors 25.

The ore dust is collected and carried by the 35 conveyors to the ore pass 30 from whence it is delivered to the cooler 31. The temperature of the calcined product flowing through the ore pass 30 is approximately 1520° F.

After being cooled, the vanadium and uranium 40 is dissolved from the calcined ore in the basic leach.

The reaction in the chamber 10 is essentially a chloridizing roast. The ore decrepitates under 45 this condition of heat in the non-oxidizing atmosphere of the drum thereby assisting reagent contact with the mineral or minerals contained in the minute interstices of the sand grains. The mineral or minerals having the power of combination are chloridized, intimately mixed with the 50 chloridizing reagent and are rendered nascent for immediate oxidation. The speed of the chemical reaction is greatly influenced by temperature, by concentration of the reacting substances and by the intimacy and amount of contact surface 55 provided in the chloridizing roast, by the cascading action and, in the oxidizing chamber, by the dispersion of the ore. The steam used to blow the ore into the oxidizing chamber becomes dissociated and forms an efficient oxidizing agent. The 60 reaction in the oxidizing chamber is that chlorine is liberated and passes off with the gases of combustion, while the sodium combines with the vanadium to form a water soluble sodium vanadate.

In the event of using sodium carbonate with the sodium chloride as reagents, a certain amount of carbonates are formed in the reducing chamber which persist throughout the roast. The CO<sub>2</sub> combines with the uranium. 5

By decrepitating the ore during chloridization, the time required for calcining is greatly reduced, the reagent contact with the vanadium and uranium is more efficient, and the mechanical features of the roaster are greatly simplified, therefore 10 both the initial cost and the operating costs are low.

The ore of the sodium chloride reagent roast is leached with water. The calcined ore renders the leaching solution basic. The soluble sodium vanadate passes into solution and is then ready for precipitation. The combined reagents, sodium chloride and sodium carbonate, when used to recover both uranium and vanadium from the ore must be treated differently in the leaching 20 of same. As above stated, a certain amount of the CO<sub>2</sub> combines with the uranium but insufficient to prevent precipitation that must be controlled. Therefore, just sufficient sodium carbonate is added to the leaching solution 25 to keep the sodium uranyl carbonate in solution, the same being soluble in an excess of sodium carbonate. The vanadium is also soluble in this solution and the two products may be selectively precipitated. By expelling the CO<sub>2</sub> of the solution, uranium will precipitate as sodium uranate. 30 The precipitation of the vanadium follows.

The machine is particularly valuable in providing an efficient treating mechanism of low initial cost and low operating cost. 35

While this invention has been described as particularly applicable to carnotite and other vanadium-uranium bearing ores for the recovery of vanadium and/or uranium values therefrom, it is not to be construed as limited to these particular 40 ores.

While a specific form of the improvement has been described and illustrated herein, it is desired to be understood that the same may be varied, within the scope of the appended claim, without 45 departing from the spirit of the invention.

Having thus described the invention, what is claimed and desired secured by Letters Patent is:

A process for treating vanadium ores to form 50 soluble vanadates comprising: the steps of forming a mixture of the ore and a salt from the class consisting of sodium chloride and sodium carbonate, subjecting the mixture in a closed drum to a heating and agitation in a non-oxidizing atmosphere, discharging the mixture from the drum 55 into an oxidation chamber, dispersing the mixture therein by a steam jet subjecting the mixture while in a dispersed condition to an oxidizing roast to convert the vanadium values therein to vanadates, collecting the roasted product and 60 leaching it to recover the vanadium values.

HARRY D. BROWN.